

## UNITED STATES PATENT OFFICE

2,261,094

## TREATMENT OF KERATINS

John Bamber Speakman, Far Headingley, Leeds,  
England

No Drawing. Application December 9, 1935, Serial No. 53,688. In Great Britain December 10, 1934

8 Claims. (Cl. 167—87.1)

This invention relates to improvements in the treatment of fibres or fibrous materials containing keratin such as hair and wool, and is particularly concerned with treatments for the application of permanent set to such substances or for the removal of stress from materials made from them, and for the treatment of keratin-containing materials in or before finishing operations.

Substances containing keratin are customarily subjected to a heat treatment, for example with steam or hot water for the application of a permanent set to fibres or for the removal of stress when in the form of fabrics. Also, it has been proposed to treat wool or hair while in the stretched condition with boiling solutions of bisulphite for the improvement of its appearance and properties and subsequently to treat the wool or hair with solutions of metal compounds such as basic alum or with oxidising agents. Treatment of wool or hair with boiling solutions of sulphites or bisulphites will cause disruption of the disulphide bond of keratin and the formation of S—NH bonds according to the following equations, where R—S—S—R and R—NH<sub>2</sub> represent the peptide and associated side chains of keratin.



The reactions take place with such readiness that the maximum possible number of linkages result and consequently a subsequent treatment with a polyvalent metal compound, organic compound or oxidising agent will not result in any appreciable rebuilding of linkages between the peptide chains of keratin.

The object of the invention is to provide a method of treatment of keratin containing substances for the removal of stress on the application of a set which may be carried out at normal or raised temperatures and which will render the keratin containing substances resistant to deterioration by alkaline media and susceptible to dyeing without the use of mordants.

The invention consists in treating fibrous substance containing keratin, such as wool or hair, with a reducing agent at such concentration, pH and temperature as to effect reduction and disruption of the constituent disulphide or cystine bond of keratin with the formation of sulphhydryl groups and thereafter treating the substance, while maintaining it in a form which it is desired

5 to render permanent, with a solution of a polyvalent metal compound or with an organic compound containing two or more reactive halogen atoms, whereby to form in or between the fibres molecules sulphur bonds containing a metal or organic grouping. The treatment with a reducing agent may be effected at normal, body or elevated temperature.

10 The disruption of the disulphide bond by reduction in this way relieves stress in the keratin-containing fibres, which stress may have been caused, for instance, by purposely deforming the fibres, as by means of a curler, and leaves the fibres in a state such that further bonds may be 15 caused to take place with the fibres in the deformed condition by subsequent treatment with the metal salt or organic compound, such bonds being —S—X—S— where X is a metal or organic grouping. The fibres are stabilised in the 20 formation which they had during such treatment and may thus be caused to take on a permanent set.

25 The bonds formed in the presence of the metal or organic compounds are resistant to steam and hot water and consequently any set or formation given to keratin-containing fibres under treatment will be retained subsequently by the fibres even in the presence of hot water and steam.

30 The resistance of keratin fibres treated according to the invention to deterioration by alkaline solutions is considerably enhanced and consequently such fibres may be subjected to treatment in alkaline liquors as in dyeing with vat or sulphur dyes without serious deterioration.

35 In order that stress may be removed from keratin containing fibres or fibrous materials, and a desired formation of the fibres or materials made permanent, it is essential that the treatment with the reducing agent to disrupt the disulphide 40 bonds should precede as a separate step the treatment with the polyvalent metal compound or organic compound. If the reducing agent and polyvalent metal compound or organic compound are employed simultaneously, reaction may take 45 place whereby the metal or organic grouping enters the disulphide bond, but the reaction takes place without change in the position of the bonds and therefore without change in the internal stress of the fibres or the formation of the fibres.

50 The metal atoms introduced into the keratin fibres by the method of the invention, moreover, may be employed for attachment of those dye molecules which ordinarily require the use of a mordant.

Examples of suitable reducing agents which

may be employed are sodium, ammonium or potassium bisulphite, sodium sulphide, sodium hydrosulphide, titanous chloride, cysteine hydrochloride, sodium hypophosphite, sodium thiosulphate, sulphurous acid, sodium hydrosulphite, ammonium, sodium or potassium sulphite, sodium dithionite and potassium metabisulphite, which may be used either alone or in combination with one another or with suitable media. The reducing agent may be formed in situ as by moistening the fibres with a small quantity of a solution of an alkali such as baryta which reacts with the fibre molecules to form a hydrosulphide, the concentration of which may be kept sufficiently high if the amount of solution employed is small.

Reducing agents as a whole, with the exception of those yielding  $\text{SO}_3^-$  ions disrupt the disulphide bond of keratin with the formation of sulphhydryl groups, although the quantity of disulphide bonds disrupted in any keratin-containing substance varies not only from one reducing agent to another, but also with the conditions of concentration, pH and temperature at which a reducing agent is employed.

The reducing agents yielding  $\text{SO}_3^-$  ions, as exemplified by sulphites, bisulphites and meta-bisulphites, effect disruption of the disulphide bond of keratin by formation of  $\text{RSNa}$  and  $\text{R}-\text{S}-\text{SO}_3\text{H}$  groupings at the boiling point, and acid sulphite solutions at pH 6 at temperatures as low as 50° C. effect the same disruption, but the formation of the groupings is immediately followed by the spontaneous formation of  $\text{SNH}$  bonds in these cases. Hence boiling solutions of reducing agents yielding  $\text{SO}_3^-$  ions and acid sulphite solutions at pH 6 at 50° C. or above cannot be employed according to the invention. At temperatures appreciably below the boiling point and as low as 37° C. solutions of bisulphites and meta-bisulphites can be employed to form sulphhydryl groups from the disulphide bonds of keratin. Under such temperature conditions the disruption of the disulphide bond is attended initially by the formation of  $\text{R}-\text{S}-\text{Na}$  and  $\text{R}-\text{S}-\text{SO}_3\text{H}$  groupings as in the case of the boiling solution but the formation of  $\text{S}-\text{NH}$  bonds does not take place. Removal of the bisulphite or meta-bisulphite from the fibres by treatment with alkali, aqueous acetone or by simple washing results in the conversion of the  $\text{R}-\text{SNa}$  and  $\text{R}-\text{S}-\text{SO}_3\text{H}$  groupings into  $\text{RSH}$  and  $\text{R}-\text{SOH}$  groups. Sufficient reducing agent is present to reduce the  $\text{R}-\text{SOH}$  groups to  $\text{R}-\text{SH}$  groups.

While the treatment of the fibres or fibrous substances containing keratin with a solution of a reducing agent may be effected within large limits of hydrogen ion concentration, it has been found that there are two conditions under which optimum results are obtained, one when the solution in contact with the hair is at about pH 6 and the other when a solution of pH 10 or above is employed.

At pH 6 the salt linkages between the peptide chains of animal fibres are most stable, relaxation in the strained fibres is delayed and more disulphide bonds remain in a state of strain for a longer time. Since many reducing agents attack strained disulphide bonds more readily than unstrained bonds, the disruption of the bonds is especially efficient at pH 6.

At or above pH 10 the reducing agents are efficient because alkalies are able to attack disulphide bonds readily whether strained or un-

strained, sulphhydryl and sulphonate acid groups being produced by hydrolysis, and the latter groups are reduced by the reducing agent to sulphhydryl groups. The sulphhydryl groups are available for combination with the metal salt or organic compound.

The metal salts employed according to the invention may be the salts of metals other than the alkali metals, examples being salts of calcium, barium, zinc, copper or nickel. The salts may be oxidizing agents, for example, nitrates, or they may be used mixed with oxidizing agents, in order that formation of disulphide bonds from sulphhydryl groups may proceed at the same time as the formation of  $\text{S}-\text{X}-\text{S}$  bonds,  $\text{X}$  being metal or an organic grouping, and thus reduce the time of treatment. Any desired concentration of the salt solutions may be employed, but 5% is a convenient concentration.

Where the solutions of reducing agents employed for disrupting the disulphide bonds are alkaline, the solutions of metal salts are desirably slightly acid in reaction, so that not only is the formation of further bonds in the fibre molecules assisted by the reduction of alkalinity in the fibres, but the probability of metal hydroxides or basic salts separating is reduced.

For the treatment of keratin-containing fibres or materials according to the invention, a solution of the reducing agent is applied to the keratin-containing fibres as by immersion of the fibres, and then after sufficient time has been allowed for reaction with the fibres, for example about 15 minutes, the solution may be removed and the fibres may be washed, or the reducing agent completely removed by the use of an agent adapted to combine with it or otherwise render it inactive, or eliminate it; for example where bisulphites are employed as reducing agents a 40 60% aqueous acetone solution may be employed to remove the agent. The washing operation or removal of the reducing agent is, however, unnecessary where the metal salt does not react with the reducing agent to form undesirable 45 compounds, such as metal sulphides, which would stain or otherwise spoil the fibres. The fibres are then treated with the metal salt care being taken to ensure that the solution reaches all the fibres. The fibres may afterwards be washed. 50 In place of a metal salt an organic compound such as phosgene may be employed to react with the reduced fibres, when disulphide linkages containing an organic grouping will be formed. If the treatment is not intended to dissipate stress 55 or impart a permanent set to deformed fibres but to form  $\text{S}-\text{X}-\text{S}$  bonds for instance to impart resistance to alkali, the fibres may be treated with a solution containing a reducing agent and a metal salt, e. g. sodium sulphite and zinc sulphate.

In carrying the invention into effect according to one method as applied by way of example to the permanent waving of human hair, the hair, after the usual shampoo, is treated with a solution of the reducing agent, e. g. sodium bisulphite, preferably of from 5 to 20 per cent. concentration, which may contain alcohol in suitable concentration, say 10%, to minimise oxidation of the bisulphite on exposure to air, and which may be warmed up to about 40° C. to assist penetration of the hair. The hair is wound on a curler and the bisulphite solution again applied, for example by admitting it into a tube surrounding the curler or by circulating it in some convenient 75 manner about the curler.

28

As an alternative method the hair may be shampooed, then wound on a curler in the dry or wet state and then have the sodium bisulphite solution applied to it while on the curler. In either case the solution is kept in contact with the hair for a period of about fifteen minutes and then withdrawn. The hair is then treated with a solution of a metal salt, e. g. 5% copper sulphate solution.

The hair may then be washed and subjected to the finishing procedure of the usual permanent waving operation.

According to another method of carrying the invention into effect for the permanent waving of human hair taking advantage of the efficiency of a reducing agent at about pH 6, a half-molar solution of sodium sulphite and bisulphite in water containing 5% alcohol is prepared, the proportions of the two compounds being adjusted to give pH 6. The solution is circulated about the hair, wound on a curler, by any convenient means for about 15 minutes, being maintained at from 35° to 50° C. or higher.

If it is not desired to circulate the reducing agent but merely to apply it to the hair before or after winding it on a curler as by means of an absorbent wad, a solution at about pH 8 is employed, since the hair reduces the pH to a value of about 6. A solution may be prepared from a half-molar solution of sodium sulphite by the addition of sodium metabisulphite or other acidic compound. When the solution is applied to the hair it rapidly decreases in alkalinity due to reaction with the hair and the pH value becomes about 6. The hair and the solution in contact therewith are preferably maintained at 35° to 50° C. or higher for about fifteen minutes, as by applying the necessary heat to the curlers or by heating the hair by a stream of hot air from a drying apparatus, evaporation of the solution being prevented in the latter case by covering the curlers or the whole head with a water-impermeable cover.

Treatment of the hair with a metal salt then follows as described above. A solution of 5% calcium or barium nitrate may be employed as the salt solution whereby both disulphide bonds are formed by oxidation of sulphhydryl groups and  $-\text{S}-\text{Ba}-\text{S}-$  or  $-\text{S}-\text{Ca}-\text{S}-$  bonds by combination of such groups with the metal.

The usual finishing procedure of ordinary permanent waving operations may then be given.

According to a modification of the above method wherein advantage is taken of the efficient disruption of disulphide bonds of keratin in reducing solutions at pH 10 or higher, a half-molar solution of sodium sulphite is brought to about pH 11 or higher by addition of sodium carbonate or sodium meta silicate, or a 6% sodium hydro-sulphide solution brought to pH 10 is employed. The solution is applied to the hair before or after winding on a curler and in addition may be circulated about the hair on the curler. A solution of an alkali, for example a baryta solution at the specified pH, may also be employed, being applied to the hair in small quantity. The alkali reacts with the hair molecules and forms a hydrosulphide. Treatment is complete in about fifteen minutes at 30° C.

A fourth normal zinc sulphate solution containing an oxidizing agent, at an equivalent concentration, and preferably acidified, is employed to form  $-\text{S}-\text{Zn}-\text{S}-$  links and in addition disulphide bonds in the fibres and thus make the set permanent. The hair may then be subjected

to the finishing treatment usual in permanent waving operations.

Successful treatment of fibres and fibrous materials may also be effected at pH values other than pH 6 and pH 10-11. Bisulphites or meta bisulphites, for example, in concentrated solutions at about pH 4 are effective in disrupting the disulphide bonds of keratin at room temperature or above. Besides disrupting the disulphide bonds the solution causes pronounced fibre swelling, being a solution of a weak acid. The effectiveness of the reagent is increased by including in solution with it an agent adapted to depress ionisation of the reagent and increase the swelling effect. Such agents are exemplified by the water soluble alcohols, ethyl alcohol, glycerol, ethylene glycol and ethyleneglycolmonomethylether.

As an example of the method of treating keratin-containing fibres in this way, a 5 to 20% solution of a bisulphite or metal bisulphite containing up to 45% ethyl alcohol is applied to unstrained hair and allowed to react for about 15 minutes at room temperature or above. The swollen hair with disulphide bonds broken is then deformed as by winding on a curler or forming the hair into curls or waves on the head, such deformation taking place without development of significant internal stress. The configuration given to the hair is then made permanent by treatment with a 5% solution of a metal salt such as copper sulphate, or a solution of an organic compound, with or without an oxidizing agent. The hair may then be given the usual finishing treatment of permanent waving operations.

In the above case the hair may equally be treated with the bisulphite or meta bisulphite solution after being deformed, as on curlers.

According to a further modification for giving hair a permanent wave or set, the hair is moistened with a solution of a reducing agent and is formed into waves or curls on the head. To facilitate manipulation of the hair a thickening agent may be added to the solution of reducing agent, for example agar agar or kieselguhr, in quantity sufficient to give the solution the consistency of a paste. Wetting agents may also be added. After treatment at room temperature or above for 15 minutes, the hair is treated with a solution of a metal salt as indicated above, and given the usual finishing treatment of permanent waving operations.

In the application of the invention to fabrics containing keratin, such as wool, the usual crabling and blowing operations for the removal or equalising of stress in the fabrics may be dispensed with and a reduction treatment in the cold or warm solutions of reducing agents, such as a 5 to 20% solution of alkali bisulphites, or a 0.6% solution of sodium sulphide given in their place. The reducing agent by disrupting the disulphide bond in the wool molecule relieves stress in the fibres. The fibres are stabilised by a subsequent treatment with a 5% or other dilute solution of a metal salt such as copper sulphate, barium chloride, zinc sulphate or nickel chloride with or without an oxidizing agent or by treatment with an organic compound such as phosphogene, an intermediate washing out of the reducing agent being given if, for example, a sulphide is used as reducing agent and the salt of a metal which forms insoluble coloured sulphides is applied for stabilising the fibres.

The invention may also be applied to the re-

70

75

moval of distortion in knitted fabrics of wool arising from uneven strain on the yarn, by treatment of the fabric with a solution of a reducing agent, and subsequent stabilising by treatment with a metal salt solution or an organic compound with or without an oxidizing agent.

Curled yarns for the manufacture of curl fabrics or artificial astrackan and Persian lamb fabrics may have a permanent set given to them by treatment of the deformed yarn with a reducing agent in the cold or warm state, followed by treatment with a solution of a metal salt with or without an oxidizing agent, to give permanence to the set.

The invention may be applied to improving the resistance of fibres or fibrous materials containing keratin, such as fabrics or yarns, to deterioration by alkalies and alkali sulphide solutions, apart altogether from the application of a permanent set to the fibre or relief of stress in the fabric, by treatment with a reducing agent, for example, as set out above, followed by treatment with a solution of a metal salt (with an intermediate washing operation where the reducing agent is liable to react with the metal salt to precipitate undesirable compounds such as metal sulphides). Keratin-containing fibres so treated may be subjected to the action of alkaline solutions as for example in vat or sulphur dyeing without appreciable deterioration. The fibres or fibrous materials in this case may be treated with a solution containing both the reducing agent and the metal salt or compound or organic compound.

As the introduction of a metal atom or other grouping into the disulphide linkages of keratin may serve for the fixing of dyes to the keratin molecules, keratin fibres or keratin-containing materials which have been treated with a solution of a reducing agent and then with a solution of a metal salt in the manner which has been described above in connection with the application of a permanent set, the release of stress or the increasing of resistance of the keratin to deterioration by alkalies, may be subjected to dyeing without the need for a preliminary mordanting operation.

I claim:

1. Method of permanently waving hair which comprises treating the hair for a period not exceeding 30 minutes with a solution of a reducing agent at a temperature appreciably below the boiling point and in the absence of amphoteric metals to effect reduction and disruption of the disulphide or cystine bond of keratin of the hair with the formation of sulphhydryl groups and thereafter treating the hair while maintaining it in a curled or waved condition with a solution of at least one polyvalent metal compound whereby to form sulphur bonds containing a polyvalent metal in the hair molecules while the hair is in the curled or waved condition.

2. Method of permanently waving hair which comprises treating the hair for a period not exceeding 30 minutes with an alkaline solution of a reducing agent at a pH of at least 10 and a temperature appreciably below the boiling point

and, in the absence of amphoteric metals to effect reduction and disruption of the constituent disulphide or cystine bond of keratin with the formation of sulphhydryl groups, and then while maintaining the hair in a curled or waved condition treating it with a solution of at least one polyvalent metal compound whereby to form sulphur bonds containing a polyvalent metal in the hair molecules while the hair is in the curled or waved condition.

3. Method of permanently waving hair which comprises treating the hair for a period not exceeding 30 minutes with a solution of at least one compound of the group consisting of acid sulphites of monovalent metals and radicals at a pH of about 4 and at a temperature substantially below the boiling point of water to effect disruption of the constituent disulphide or cystine bond of keratin of the hair with the formation of sulphhydryl and S-sulphonic acid groups, and then while maintaining the hair in a curled or waved condition treating it with a solution of at least one polyvalent metal compound, whereby to form sulphur bonds containing a polyvalent metal in the hair molecules while the hair is in the curled or waved condition.

4. Method as claimed in claim 1 wherein the hair is treated with the reducing agent and, in the form of strands, is then wound on curlers and treated with a solution of at least one polyvalent metal compound while on the curlers.

5. Method as claimed in claim 2 wherein the hair is treated with the reducing agent and, in the form of strands, is then wound on curlers and treated with a solution of at least one polyvalent metal compound while on the curlers.

6. Method as claimed in claim 3 wherein the hair is treated with the acid sulphite and is then wound on curlers in the form of strands, and is treated with the solution of at least one polyvalent metal compound while on the curlers.

7. Method of permanently waving hair which comprises treating the hair with an alkaline solution of an organic hydrosulphide, in the absence of amphoteric metals, to effect disruption of the disulphide bond of keratin of the hair and then while maintaining the hair in a curled or waved condition treating it with a solution of at least one polyvalent metal salt whereby to form sulphur bonds containing a polyvalent metal in the hair molecules while the hair is in the curled or waved condition.

8. Method of permanently waving hair which comprises treating the hair for a period not exceeding 30 minutes with an alkaline solution of a hydro-sulphide of an alkali metal, including ammonium, at a pH of at least 10 and at a temperature appreciably below the boil, in the absence of amphoteric metals, to effect disruption of the disulphide bond of the keratin of the hair and then while maintaining the hair in a curled or waved condition treating it with a solution of at least one polyvalent metal salt whereby to form sulphur bonds containing a polyvalent metal in the hair molecules while the hair is in the curled or waved condition.

JOHN BAMBER SPEAKMAN.